

Oct. 6, 1942.

J. K. ELY

2,298,113

LIGHTWEIGHT ELECTRIC IRON

Filed Dec. 7, 1940

Fig. 1.



Fig. 2.



Fig. 3.



Fig. 4.



WITNESSES:

C. J. Weller.  
K. C. Kepler.

INVENTOR  
James K. Ely.

BY  
W. C. Coley  
ATTORNEY

## UNITED STATES PATENT OFFICE

2,298,113

## LIGHTWEIGHT ELECTRIC IRON

James K. Ely, Wilkinsburg, Pa., assignor to Westinghouse Electric & Manufacturing Company, East Pittsburgh, Pa., a corporation of Pennsylvania

Application December 7, 1940, Serial No. 369,020

3 Claims. (Cl. 38—93)

This invention relates to pressing or sad-irons and, more particularly, to lightweight irons.

Since a pressing or sad-iron must be moved by the hand of an operator, usually a housewife or maid, there has been a universal demand for a really lightweight sad-iron. Various ingenious attempts have been made and are being made to reduce the weight of the present well-known irons. Most of these attempts have failed to produce the desired light-weight iron because the sole plate employed was formed from cast iron.

In other irons, aluminum has been employed as the sole plate or ironing surface, but these irons have not proven to be satisfactory commercially as they are easily dented and marred. Where precipitation hardened aluminum alloy sole plates are employed, it is found that they cannot retain their hardness at the high operating temperatures of about 250° C. to 325° C. and are, therefore, easily marred and the flat ironing surface destroyed in a very short time under the blows and other conditions encountered in normal service.

Other irons have been produced having an aluminum sole plate to which a chromium coating has been electrolytically applied. Heretofore, the aluminum irons having a chromium ironing surface have failed in a relatively short period of time because the chromium surface did not permanently adhere to the aluminum sole plate. Instead, it is found that slight blows, such as are encountered in service, destroy the bond between the sole plate and the chromium plating with the result that the chromium plate blistered and peeled unevenly over the surface of the sole plate. It is thought that one of the reasons for the failure of these aluminum irons was that the aluminum metal utilized as the sole plate is so soft or where a precipitation hardened aluminum alloy is employed, becomes so soft under the operating temperatures encountered, as to fail to provide a sufficiently hard backing for the chromium plate.

It is, therefore, desired to produce a lightweight iron, preferably of aluminum or aluminum base alloys, which will withstand the usual rough treatment given an iron and which has an ironing surface formed of an exterior metallic plating so bonded thereto as to prevent blistering or peeling thereof while at the same time providing a sufficiently hard backing for the metallic plating that the iron will maintain these desirable characteristics during operation over a wide range of temperatures.

It is, therefore, an object of this invention to

provide a lightweight aluminum base iron having an inexpensive, easily applied, hard backing layer for the metallic iron surface, the backing layer functioning to tenaciously bond the metallic ironing surface to the aluminum base, thereby providing a permanent hard glossy exposed ironing surface irrespective of the operating temperature of the iron.

Another object of this invention is to provide a lightweight iron of aluminum or aluminum base alloy having a chromium ironing surface bonded thereto by means of a hard backing layer composed of an oxide.

Another object of this invention is to provide a lightweight iron of aluminum or aluminum base alloy having a chromium ironing surface bonded thereto by means of intermediate layers composed of a hard backing layer of an oxide and a layer of nickel electrolytically deposited thereon.

Other objects of this invention will become apparent from the following description when taken in conjunction with the accompanying drawing, in which:

Figure 1 is a perspective view of an iron embodying this invention;

Fig. 2 is a transverse sectional view of the iron shown in Fig. 1;

Fig. 3 is a fragmentary sectional view taken along the line III—III of Fig. 2; and

Fig. 4 is a view similar to Fig. 3 illustrating another embodiment of this invention.

Referring to the drawing, in which like reference characters indicate like parts in the several figures, an iron structure 10 is illustrated comprising a lightweight aluminum or aluminum alloy base or sole plate 12 and an electric heating element 14 disposed therein for heating the sole plate. The heating element 14, while being shown as cast or embedded within the sole plate 12 may, however, be associated with the base 12 in any other desired manner. The operation of the electric heating element 14 is selectively controlled by a thermostat 16 in a well known manner.

In accordance with this invention, the aluminum or aluminum alloy sole plate 12 is provided with an exterior hard lustrous coating forming the ironing surface, as will be explained more fully hereinafter. Since the aluminum sole plate 12 is inherently relatively soft and easily dented, the iron surface is formed of a plurality of layers of suitable material for increasing the scratch and dent resistance of the sole plate during normal usage of the iron.

Referring to Fig. 3 of the drawing, there is

illustrated a preferred embodiment of this invention in which a hard backing layer 18 is applied to the aluminum or aluminum alloy base 12, after which a layer of chromium 20 is applied to the backing layer 18 for providing the desired hard and lustrous ironing surface.

The layer 18 is preferably formed of aluminum oxide deposited in any desired manner such as, for example, by anodizing the sole plate in oxalic acid for a given period of time. The method of forming the anodized aluminum layer 18 need not be described in detail however, since different methods are well known in the art and by themselves form no part of the present invention. The layer 18 formed by any of the well known commercial anodizing methods is quite hard and is so bonded thereto as to be an integral part of the aluminum sole plate 12 so that there is no danger of breaking the bond between the layer 18 and the sole plate 12. In addition to being quite hard, it is found that the anodized layer 18 provides an ideal medium for electroplating the exterior metallic coating 20 of chromium thereto.

The metallic layer 20 of chromium is applied to the layer 18 of anodized aluminum by any suitable method of electroplating, it being found upon a close examination of the resulting plate that the chromium plated on the layer 18 actually penetrates the minute interstices formed between the various flakes of oxide giving a definite bond with the layer 18. The thickness of the exterior chromium coating 20 may be of any magnitude desired, it being understood that the greater the thickness of the chromium plate the greater the resisting power of the composite layers forming the ironing surface to denting.

In practice, after the chromium plate has been formed and securely bonded to the intermediate anodized layer, the exterior surface is buffed to a high lustrous condition in any of the well known manners to provide an attractive serviceable iron. The combination of the backing layer 18 of the anodized aluminum and the exterior coating of chromium cooperate to provide a very hard, dent and scratch resisting ironing surface on the aluminum sole plate, while at the same time permanently adhering to the sole plate.

In another embodiment of this invention as illustrated in Fig. 4, an intermediate layer 22, preferably nickel, is electrolytically deposited between the layers 18 and 20 of anodized aluminum and chromium, respectively, for providing a thicker scratch resisting ironing surface on the sole plate 12. The thickness of the layer 22 of nickel in this embodiment may vary, it being found that the thicker the nickel layer, the more resistant the ironing surface is to denting. Where desired, the layer 22 of nickel may be employed as the exterior ironing surface, the exterior surface being buffed in the usual manner to provide the smooth highly lustrous exterior surface. Whether the nickel layer is employed as the exterior ironing surface or as an intermediate layer between the anodized layer 18 and the exterior layer 20 of chromium, it is found that the layer 18 of the anodized aluminum cooperates with the exterior surface to give the desired hard backing layer while at the same time permanently bonding the adjacent layer to the sole plate 12.

Since the iron of this invention utilizes a sole plate of aluminum or aluminum alloy, it is quite apparent that the iron will function efficiently to transmit the heat from the heating element to the ironing surface of metallic plating formed

on the sole plate. This can readily be appreciated when it is considered that aluminum has a thermal conductivity of approximately 33% or about four times that of the cast iron bases employed heretofore. In addition to having a good thermal conductivity, the resulting iron is extremely lightweight by reason of the metals employed in its construction. Further, because of the backing layer of anodized metal, the resulting iron has an ironing surface which is resistant to denting and scratching during normal usage of the iron, while at the same time retaining its desired characteristics throughout operating temperatures of up to as high as about 325° C.

Throughout the description given hereinbefore aluminum and aluminum base alloys are considered as equivalents and where the term aluminum is employed in the appended claims it is intended to include both aluminum and aluminum base alloys.

Although this invention has been described with reference to a particular embodiment thereof, it will be obvious to those skilled in the art that it is not to be so limited but is susceptible of various changes and modifications without departing from the spirit thereof and that it is, therefore, not to be limited except insofar as such limitation shall be placed thereon as are specifically set forth in the appended claims.

I claim as my invention:

1. An iron comprising an aluminum base having a working surface, means to heat said base member operatively associated therewith, a layer of adherent anodized aluminum integrally formed on at least the working surface of the base of the iron, and an exterior metallic coating electroplated upon the layer of anodized aluminum on at least the working surface, the electroplated coating being integrally bonded throughout the electroplated area with the layer of anodized aluminum, the layer of anodized aluminum cooperating with the exterior metallic coating to strengthen the exterior coating and render it resistant to physical shock, the bond between the layer of anodized aluminum, the aluminum base and the exterior metallic coating being so adherent and so resistant to thermal shock that it is capable of withstanding repeated heating to high temperatures without detrimental effect thereon.

2. An iron comprising an aluminum base having a working surface, means to heat said base member operatively associated therewith, a layer of adherent anodized aluminum integrally formed on at least the working surface of the base of the iron, and an exterior layer of chromium electroplated upon the layer of anodized aluminum on at least the working surface, the layer of chromium being integrally bonded throughout the electroplated area with the layer of anodized aluminum, the layer of anodized aluminum cooperating with the layer of chromium to strengthen the exterior layer and render it resistant to physical shock, the bond between the anodized aluminum and each of the base and layer of chromium being so adherent and so resistant to thermal shock that it is capable of withstanding repeated heating to temperatures of up to about 325° C. without detrimental effect thereon.

3. A lightweight hand iron comprising, in combination, an aluminum base member having a lower surface, means to heat said base member operatively associated therewith, a layer of anodized aluminum integrally and adherently

formed on at least the lower surface of the base member, a layer of nickel electroplated upon the layer of anodized aluminum on at least the lower surface of the base member, and a layer of chromium electroplated upon the layer of nickel on at least the lower surface of the base member, the electroplated layers being integrally bonded to each other and to the anodized aluminum throughout the entire electroplated areas, the layer of nickel and the layer of anodized alumi-

num cooperating to provide a hard dent resisting medium to strengthen the layer of chromium and render it resistant to shock, the bond between the different layers and the lower surface being so secure and resistant to thermal shock as to withstand repeated heating to temperatures of up to about 325° C. without detrimental effect thereon.

JAMES K. ELY.